

## 1

3,092,506

## WAX COMPOSITIONS

Anna M. Shadan, Ponca City, Okla., assignor to Continental Oil Company, Ponca City, Okla., a corporation of Delaware

No Drawing. Filed July 26, 1960, Ser. No. 45,293

10 Claims. (Cl. 106—270)

This invention relates to wax compositions useful in surface coating applications generally and especially adapted for the coating or lining of paper containers and the like wherein combustibles are temporarily stored. More particularly, this invention concerns paraffin wax compositions containing a minute amount of an oil-soluble petroleum sulfonate soap which compositions in the molten or fluid state exhibit improved non-foaming tendencies. The present invention further relates to a process for preparing said wax compositions.

Because of their outstanding resistance to water and overall excellent chemical resistance and inertness, waxes are extensively utilized to coat paper containers designed for packaging combustibles. Probably the most notable example of an application of this type is exemplified in the packaging of dairy products, particularly milk. In carrying out the coating procedure, it is customary to dip a flat blank of the carton container into a molten bath of the wax and thereupon shape the blank after the wax deposit has suitably solidified.

Most waxes, irrespective of their source or origin, exhibit objectionable foaming tendencies in the molten state, especially when liquid baths thereof are subjected to the degree of mechanical agitation normally occurring in the various coating operations. Generally, the character of the foam encountered in molten wax compositions is sufficiently stable so that when the wax solidifies on the surface of the paper there results portions thereof having thin or otherwise inadequate covering of the wax. If these faulty areas are on the surface forming the inside of the container, it is likely that the liquid contents will ultimately penetrate the paper at these areas thereby weakening the paper to the extent that leakage develops. On the other hand if the foam covers the outside of the container, the functional purpose of the container may not be adversely affected but nevertheless in many of such instances the containers have to be disposed of as rejects because of their unattractive appearance.

In current commercial wax coating practices of the type hereinabove mentioned a petroleum, and more specifically, a paraffin wax is favored since this type of wax is readily available and comparatively inexpensive. This invention, however, is not limited to the use of a petroleum wax but can be beneficially utilized to inhibit the foaming tendencies of other type waxes and mixtures thereof with a petroleum wax.

One of the principal objects of the present invention is to provide a non-foaming wax composition.

Another object of this invention is to provide a paraffin wax composition containing a small but effective amount of an oil-soluble sodium salt of a petroleum sulfonate capable of rendering said composition substantially non-foaming in nature when existing in a molten state.

Other objects and advantages of this invention will become more apparent to those skilled in the art upon a consideration of the detailed discussion and example set forth hereinbelow.

Since paraffin wax or a wax composition containing a major portion of paraffin wax is viewed as the preferred composition in the practice of this invention, a mention will be made here to the various grades and types coming within the scope of the term "paraffin wax" as contemplated herein. This can be best accomplished by briefly

## 2

considering the procedures ordinarily involved in producing a paraffin wax.

Paraffin waxes are the wax constituents occurring in various fractions of certain crude petroleums. They manifest melting points in a range of about 47 to 65° C. and Saybolt viscosities in the range of from about 35 to 45 S.U. at 210° F., and are further physically characterized by crystallizing into large, well-formed distinct crystals of the plate and needle types. The precise physical characteristics of a paraffin wax may vary depending upon the crude source, the portion of the crude used for wax production and differences in refining techniques.

In the preparation of paraffin wax, a crude petroleum stock having such a wax constituent is subjected to fractional distillation whereby cuts are obtained ranging from heavy gas oil to heavy lubricating oil. The light fractions or cuts are the richest in wax components and accordingly are usually termed paraffin or wax distillates. These paraffin rich fractions are normally liquid at 80 to 100° F., whereas cooling below this range readily effects precipitation of the wax. This limited solubility characteristic at low temperatures is availed of to segregate most of the wax content. The precipitate is then filtered by any of several conventional methods in a process termed pressing which process yields a filtrate called slack wax. Slack wax normally contains from about 20 to 40% oil content. Subsequent to the pressing operation, the slack oil is "sweated." Sweating is accomplished by heat treating the slack wax whereby the oil will drain or sweat out of the solid wax as the temperature is slowly raised. The sweating operation yields a crude scale wax containing about 2% oil and melting at about 122–124° F. Fully refined paraffin wax is then obtained by merely further sweating the crude scale wax to a specific melting point range followed by treatment with a suitable adsorbent such as fuller's earth, bone char, bauxite and the like. The fully refined product is substantially free of oil.

The use of the highly refined type of paraffin wax is not mandatory in the various coating operations mentioned hereinabove. Thus, mixtures of the refined product with slack wax or crude scale wax may be advantageously employed. Furthermore, substantial amounts of other wax materials may be incorporated in the paraffin wax in order to obtain certain desired properties relating to tensile strength, melt characteristics, etc. For example, the paraffin wax can be mixed with synthetic materials such as the wax-like amorphous polyethylenes or polypropylenes, pentaerythritol esters, and the like. Additionally, waxes of animal or vegetable origin can be similarly used, e.g., beeswax, carnauba wax, etc. Also, microcrystalline waxes can be advantageously used in combination with paraffin wax.

It is also contemplated that non-wax additives can be included in the wax composition such as, for example, an anti-oxidant capable of inhibiting any oxidation tendency of the wax or waxes present.

In view of the above, the term "paraffin wax composition" used herein and in the appended claims broadly contemplates those above-described compositions or mixtures having general utility in the coating arts. However, a preferred wax composition for practicing the present invention is one wherein the paraffin wax content is at least 50% of the total weight of the composition.

In accordance with the present invention, foaming tendencies of a paraffin wax composition can be substantially and in many instances completely eliminated by homogeneously incorporating thereinto relatively minute quantities of a sodium salt of an oil-soluble or mahogany sulfonate. I have found unexpectedly that a comparatively small but characterizable class of the aforesaid sulfonates will effectively stabilize a molten paraffin wax composition containing at least about 50% paraffin wax against foam

formation. Not only are these sulfonates excellent arresters of foaming tendencies in said environment but the chemical nature thereof and the small quantities needed in order to secure beneficial stabilization are such which do not significantly affect the nontoxicity characteristics of the paraffin wax composition. This obviously is very important since these wax compositions are extensively used to coat paper containers which ultimately come into contact with food.

As indicated above, only a particular type of mahogany sulfonate can be used effectively in the practice of this invention. There are several ways of empirically classifying the different mahogany sulfonates generally available such as by average molecular weight, relative solubility in oil, etc. However, there are considerable shortcomings to this manner of defining the particular class of sulfonates useful herein and accordingly it has been noted that the most satisfactory method of characterizing these suitable sulfonates consists of specifying the particular type or fraction of petroleum oil from which the present sulfonates can be derived.

The sulfonates which I have found to be effective anti-foamants for paraffin wax compositions are those oil-soluble products obtained by sulfonating a petroleum oil fraction having a viscosity between about 80 and 120 Saybolt Universal seconds at 100° F. The preferred sulfonates are those derived from a petroleum fraction having a viscosity of about 100 SUS. Suitable fractions can be obtained from any of the paraffinic, naphthenic, or mixed base crudes. Depending on the particular type of crude source used to obtain this fraction, it may be desirable to vary the sulfonation procedure. Thus, the conventional procedure is used when employing a paraffinic base crude, namely, of solvent refining the crude employing only one solvent extraction step and thereupon sulfonating the raffinate. In other instances where a fraction is employed which had been obtained from a crude containing a high content of aromaticity, it is generally desirable to treat the fraction with two or more solvent extraction steps before subjecting the final raffinate to a sulfonation procedure. The solvent refining step or steps facilitate separation of excessive amounts of the aromatic hydrocarbons from the lubricating oil fraction which hydrocarbons if allowed to remain complicate recovery of the desired sulfonates. The various types of extracting agents which can be used are such as furfural, liquid sulfur dioxide, etc. Ordinarily furfural is preferred as the solvent extracting agent.

In sulfonating the raffinate any of the conventional sulfonating agents and techniques can be used. Suitable among the sulfonating agents are: concentrated sulfuric acid, fuming sulfuric acid (oleum), sulfur trioxide, chlorosulfuric acid, etc. Fuming sulfuric acid compositions containing from about 10 to 50% by weight excess SO<sub>3</sub> represent the preferred sulfonating agents.

Sulfonation temperatures are usually controlled within the range of about 50 to 200° F. with the preferred operating range being between about 80 and 160° F. The oil-acid weight ratio varies with the sulfonation temperature, the extent to which the lubricating oil fraction has been refined, etc., but generally is in the range from about 1.5 to 6 when using the preferred sulfonating agents.

The sulfonation step produces two principal types of sulfonation products. One type, termed green acids, are water soluble and settle out of the sulfonation reaction system as a sludge. The desired oil soluble or mahogany sulfonates remain in the oil phase and are appropriately recovered for the purposes herein by neutralizing the dissolved acids with sodium hydroxide and then extracting the resulting salts by means of a dilute aqueous solution of an alcohol such as isopropanol.

The amount of the oil-soluble sodium sulfonate which can be used in order to stabilize paraffin waxes against foam formation in accordance with this invention is a variable and ranges from about 0.01 to 0.1% based on the

weight of the wax composition. Quantities greater than 0.1% can be used to attain foam stabilization, however, the use of amounts significantly greater than this stated maximum figure may cause a condition of blistering when a paper substrate is coated with a wax containing such amounts of the sodium sulfonate. A preferred amount of sulfonate ranges between about 0.02 and 0.05% based on the weight of the wax composition.

Various ways can be employed to effectively incorporate the instant anti-foamants into the wax composition. The sulfonate can be incorporated directly into the molten wax by means of a high speed stirrer or similar device. However, because of the high viscosity associated with the instant sulfonates, it is preferred to blend same with a white mineral oil and thus incorporate these mixtures into the molten wax composition. Using this mode of incorporation, applicable ratios of sulfonate to white mineral oil can vary from about 7:3 to 1:9, respectively.

In order to further illustrate the nature of the present invention the following example is given in which all parts or percent figures are by weight. It is to be understood that this invention is not limited to the specific details set forth in this example except that such limitations are expressed in the appended claims.

#### EXAMPLE I

This example illustrates the effectiveness of a sodium salt of a mahogany sulfonate obtained from a petroleum oil having a viscosity of about 100 SUS as an anti-foaming agent for a wax composition. The wax used in the series of tests outlined below was a paraffin wax having a melting point of about 127-128° F. modified with 15% of a micro-crystalline wax.

A specimen of standard stock paper used to prepare milk cartons was provided with a coating of wax by immersing the paper within a bath of the molten wax. Upon withdrawing the specimen and solidification of the applied coating the specimen was noted for uniformity of coating and rated accordingly. These ratings were based on numerical value given on a demerit scale ranging from zero to eight. In this particular system of rating, seven indicates an excessive amount of faults due to foam. On the other hand, a rating of zero indicates that the coating is substantially free of any irregular portions attributed to the presence of foam within the coating bath. In general, ratings of four or less indicate that the coating is acceptable.

Additionally each of the tests includes a rating for blistering which is set forth as being either satisfactory or unsatisfactory.

The composition of the various wax coating baths together with the respective ratings noted therefor are set forth in the following Table I. In all tests, with the exception of the control and that identified as coating F, the anti-foaming agent was incorporated into the molten wax as a dispersion of the soap in white mineral oil in the ratio of 7:3, respectively.

Table I

|                        | Percent Anti-Foamant <sup>1</sup> | Foam Rating | Blistering                          |
|------------------------|-----------------------------------|-------------|-------------------------------------|
| Coating A (Control)    | 0.0                               | 7           | Satisfactory.                       |
| Coating B              | 0.01                              | 4           | Do.                                 |
| Coating C              | 0.02                              | 2           | Do.                                 |
| Coating D              | 0.03                              | 1           | Do.                                 |
| Coating E              | 0.04                              | 1           | Do.                                 |
| Coating F <sup>2</sup> | 0.0                               | 7           | Do.                                 |
| Coating G              | 1.0                               | 1           | Unsatisfactory (Severe blistering). |

<sup>1</sup> Sodium salt of a mahogany sulfonate having a M.W. of about 435 obtained from a solvent extracted lube oil fraction of 100 SUS at 100° F.

<sup>2</sup> Contains 1% added white mineral oil.

I claim:

1. A paraffin wax composition stabilized against foam formation in the molten state consisting essentially of a

paraffin wax containing a homogeneous dispersion of a small but effective foam inhibiting amount of a sodium salt of a mahogany sulfonate obtained by contacting a petroleum oil fraction having a viscosity between about 80 and 120 SUS at 100° F. with a sulfonating agent.

2. A paraffin wax composition stabilized against foam formation in the molten state consisting essentially of a paraffin wax containing a homogeneous dispersion of from about 0.01% to 0.1% of a sodium salt of a mahogany sulfonate obtained by contacting a petroleum oil fraction having a viscosity between about 80 and 120 SUS at 100° F. with a sulfonating agent.

3. A paraffin wax composition stabilized against foam formation in the molten state consisting essentially of a paraffin wax containing a homogeneous dispersion of from about 0.02% to 0.05% of a sodium salt of a mahogany sulfonate obtained by contacting a petroleum oil fraction having a viscosity between about 80 and 120 SUS at 100° F. with a sulfonating agent.

4. A paraffin wax composition stabilized against foam formation in the molten state consisting essentially of a paraffin wax containing a homogeneous dispersion of from about 0.01% to 0.1% of a sodium salt of a mahogany sulfonate obtained by contacting a petroleum oil fraction having a viscosity of about 100 SUS at 100° F. with a sulfonating agent.

5. A paraffin wax composition stabilized against foam formation in the molten state consisting essentially of a paraffin wax containing a homogeneous dispersion of from about 0.02% to 0.05% of a sodium salt of a mahogany sulfonate obtained by contacting a petroleum oil fraction having a viscosity of about 100 SUS at 100° F. with a sulfonating agent.

6. A paraffin wax composition comprising at least about 75% paraffin wax, said composition containing a homogeneous dispersion of from about 0.02% to 0.05% of a sodium salt of a mahogany sulfonate obtained by

35

contacting a petroleum oil fraction having a viscosity between about 80 and 120 SUS at 100° F. with a sulfonating agent.

7. A paraffin wax composition comprising at least about 75% paraffin wax, said composition containing a homogeneous dispersion of from about 0.02% to 0.05% of a sodium salt of a mahogany sulfonate obtained by contacting a petroleum oil fraction having a viscosity of about 100 SUS at 100° F. with a sulfonating agent.

8. A process for stabilizing a paraffin wax composition against foam formation in the molten state comprising uniformly admixing with said composition from about 0.01% to 0.1% of a sodium salt of a mahogany sulfonate obtained by contacting a petroleum oil fraction having a viscosity between about 80 and 120 SUS at 100° F. with a sulfonating agent.

9. A process for stabilizing a paraffin wax composition against foam formation in the molten state comprising uniformly admixing with said composition from about 0.02% to 0.05% of a sodium salt of a mahogany sulfonate obtained by contacting a petroleum oil fraction having a viscosity of about 100 SUS at 100° F. with a sulfonating agent.

10. A process for stabilizing a paraffin wax composition containing at least about 75% paraffin wax against foam formation in the molten state which comprises uniformly admixing with said composition from about 0.02% to 0.05% of a sodium salt of a mahogany sulfonate obtained by contacting a petroleum oil fraction having a viscosity between about 80 and 120 SUS at 100° F. with a sulfonating agent.

References Cited in the file of this patent

UNITED STATES PATENTS

|           |          |       |               |
|-----------|----------|-------|---------------|
| 2,009,345 | Schrauth | ----- | July 23, 1935 |
| 2,796,355 | Higgins  | ----- | June 18, 1957 |